# EUROPEAN PATENT SPECIFICATION

(11) **EP 3 902 953 B1**
(45) Date of publication and mention of the grant of the patent: **27.11.2024**
(21) Application number: 19828777.3
(22) Date of filing: 20.12.2019
(51) Int. Cl.: D06M 11/46, D06M 23/08, D06P 1/44

(54) **PROCESS FOR PRODUCING TEXTILE ARTICLES AND TEXTILE ARTICLES OBTAINED THEREFROM**
VERFAHREN ZUR HERSTELLUNG VON TEXTILARTIKELN UND DAMIT HERGESTELLTE TEXTILARTIKEL
PROCÉDÉ DE PRODUCTION D'ARTICLES TEXTILES ET ARTICLES TEXTILES AINSI OBTENUS

(30) Priority: 28.12.2018 EP 18248276
(43) Date of publication of application: 03.11.2021
(73) Proprietor: Sanko Tekstil Isletmeleri San. Ve Tic. A.S., 16400 Inegol - Bursa (TR)
(72) Inventor: LOYAN, Kenan, 16400 Inegol - BURSA (TR); HAMITBEYLI, Agamirze, 16400 Inegol - BURSA (TR); OZDEN, Erdogan Baris, 16400 Inegol - BURSA (TR); AKDAG, Hatice Aybige, 16400 Inegol - BURSA (TR); AKAR, Seren, 16400 Inegol - BURSA (TR); ZEYREK, Mustafa, 16400 Inegol - BURSA (TR); SEN, Murat, 16400 Inegol - BURSA (TR); AKBULUT, Sabrettin, 16400 Inegol - BURSA (TR)
(74) Representative: Gislon, Gabriele
(86) International application number: PCT/EP2019/086862
(87) International publication number: WO 2020/136148

(56) References cited:
- EP-A2- 0 073 090
- EP-A2- 0 105 598
- WO-A1-03/008699
- CN-A- 105 755 800
- GB-A- 1 391 593
- GB-A- 2 051 163
- JP-A- H04 136 273
- DATABASE WPI Week 200739, 2007 Derwent World Patents Index; AN 2007-408461, XP002791267
- DATABASE WPI Week 200260, 2002 Derwent World Patents Index; AN 2002-561635, XP002791268

## Description

### Field of the invention

The present invention relates to the field of textiles, in particular to a process for producing treated textile articles and to textiles articles obtained through the process. The process of the invention increases opacity of textile articles. The present invention also relates to compositions that are suitable to impart opacity to textiles to which they are applied, and that are suitable to be used in the mentioned process.

### Background of the invention

White garments and apparels are appreciated by consumers and highly requested on the market.

However, white garments and apparels have some drawbacks.

For example, white garments generally reveal the colour of the skin and/or the colour and the shape of the underwear of the user when the garments are worn.

To overcome this drawback, heavy fibres or yarns, and/or tight weavings of the yarns can be used to obtain substantially opaque, non-transparent fabrics and garments. However, this solution allows for the production of a very limited variety of garments and clothing article, i.e., garments having, for example, a weight range below which the problem appears again.

Generally, titanium dioxide is provided to fabrics to impart anti-UV, antibacterial and self-cleaning properties. It is also known to apply titanium dioxide or a composition containing TiO₂ to fabrics to obtain opaque white garments.

KR910006104(B1) discloses a process for the preparation of an opaque fibre textile. A fabric which is composed of polyester filament yarns is impregnated with a solution composed of titanium dioxide 4-7% and dispersing agent 0.1-0.5% by weight of treated fabric. Titanium dioxide has particle diameter 0.1-0.4 µm. The solution is applied by impregnation for 20-30 minutes, and fixed to the fabric. The treated fabric is then coated with a transparent resin, where the main component is diisocyanate.

However, the process disclosed in KR910006104(B1) requires two separate steps, i.e., a step of impregnation of the fabric with the titanium dioxide, and a second step of coating with resin. Therefore, the process disclosed in KR910006104(B1) is a complex manufacturing process which, additionally, requires long working time. Moreover, the resin coating, which covers the titanium dioxide, may provide an unpleasant aesthetical appearance to the fabric, and thus to the garments comprising it.

GB2051163 discloses a method of preparing an opaque fabric by increasing its covering power with TiO₂.

WO03/008699 discloses a material system and method for protecting yarns, fibers, fabrics and finished textiles from deleterious effects of ultraviolet radiation. The system comprises a material including: (i) at least one physical UVR attenuator, having average particle size below 1000 nanometers; (ii) at least one chemical UVR attenuator, and (iii) at-least one flexible, film-forming polymeric binder for bonding said material to a textile surface. The physical UVR attenuator can include titanium dioxide, zinc oxide or polytetrafluoroethylene.

JPH04136273A discloses an opacifying agent for polyester fiber knitted or woven fabrics, comprising an aqueous dispersion obtained by dispersing titanium dioxide and a polyester polyether resin in water.

DATABASE WPI, Week 200739, 2007Thomson Scientific, London, GB; AN 2007-408461 XP002791267, -& JP 2007 092221 A (NIKKA KAGAKU KK) 12 April 2007 (2007-04-12), discloses a method for producing an opaque fiber that includes applying an aqueous dispersion containing titanium oxide and a polyurethane resin to a fiber material, wherein the polyurethane resin contains (a) a polyisocyanate and (b) a polyol.

DATABASE WPI, Week 200260, 2002Thomson Scientific, London, GB; AN 2002-561635 XP002791268, -& JP 2002 161473 A (UNICHIKA TEXTILE KK) 4 June 2002 (2002-06-04), discloses a fiber with solar heat-shielding properties that comprises two or more kinds of inorganic group compound particles or organic group compound particles having different refractive indices fixed on the fiber. Inorganic pigments such as titanium oxide (anatase type or rutile type), zinc oxide, zinc sulfide, silica, alumina, white carbon, and the like may be used as inorganic compound particles.

Also, opaque white fabrics known in the art generally start to undergo a progressive reduction of their whiteness grade after a few home washings.

### Summary of the invention

It is an aim of the present invention to solve the above mentioned problems and to provide a process for increasing opacity of fabrics, especially of white or light coloured fabrics.

Still another aim of the present invention is to provide a process which allows to increase the whiteness of fabrics.

A further aim of the present invention is to provide a fabric which is white or has a light colour and substantially hides the skin and body of the user, or hides the colour and shape of his underwear, when a garment including said fabric is worn by the user.

These and other aims are achieved by the process according to claim 1, which is, thus, an object of the present invention.

Another object of the present invention is a fabric according to claim 17.

Still further objects of the present invention are a garment according to claim 23, comprising the said treated fabric, an aqueous composition according to claim 24, and the use of said composition in the process of the invention, according to claim 26.

### Brief description of the drawings

- Figure 1A and Figure 1B are photographs showing a sample fabric before (Figure 1A) and after (Figure 1B) the process of the invention.
- Figure 2A and Figure 2B are magnified photos at 10X that show a sample fabric before (Figure 2A) and after (Figure 2B) the process of the invention.
- Figure 3A and Figure 3B are photographs taken at magnification of 60X that show a sample fabric before (Figure 3A) and after (Figure 3B) the process of the invention.

### Detailed Description

In the following description, the features of the invention will be described with reference to exemplary embodiments; however, any feature of the invention disclosed herein, may be combined with one or more other features here disclosed to provide further embodiments of the present invention. Such embodiments shall be considered as disclosed by the present application.

As above mentioned, an object of the present invention is a process for producing a treated fabric, comprising the step of:
a) providing at least a fabric,
b) treating at least part of the fabric with an aqueous composition comprising titanium dioxide and at least a binder, preferably a crosslinkable binder, and
c) heating the fabric obtained in step b);
wherein said binder has a glass transition temperature (Tg) in the range from -30°C to 0°C, wherein glass transition temperature (Tg) is measured according to ASTM E1356, and/or a Shore A hardness that is ≤ 30° Shore A, wherein Shore A hardness is measured according to ASTM D2240.

Advantageously, the process of the invention allows for the production of textiles that are suitable to be used in the production of white garments, for example light weight white garments. In fact, it has been surprisingly observed that, through the process of the invention, opacity of fabrics can be increased, whilst maintaining the textiles white, soft and stylish.

In other words, it has been observed that, through the process of the invention, the transparency of a fabric can be reduced, so that the skin and the underwear of the user can no longer be seen "through" a white fabric apparel, when a garment comprising the invention fabric is worn. Transparency is here used to identify the fact that medium-light white fabrics are not opaque enough to prevent the colours and shape of skin/underware to be revealed. In other words, the said fabrics have a low covering power.

In particular, it has been observed that the titanium dioxide of the composition adheres to yarns and fibers of the fabric. Additionally, it has been observed that, when a fabric is treated according to the process of the invention, titanium dioxide is also located between at least part of the yarns of the fabric, e.g., between the weft and warp yarns of a woven fabric, thus providing for a reduction of transparency, with respect to the untreated fabric. For example, in a fabric obtainable according to the invention, titanium dioxide and the binder are also located in the spaces defined by two adjacent warp yarns and two adjacent weft yarns that float over or under said warp yarns.

Also, advantageously, the process of the invention allows to increase the whiteness and the covering power of fabrics, with respect to untreated fabrics.

According to embodiments, fabrics suitable to be used according to the present invention are preferably not dyed.

According to the process of the invention, an aqueous composition comprising titanium dioxide and at least a binder, preferably a crosslinkable binder, is provided to at least part of a fabric. In embodiments, the binder is a compound, e.g. a polymer, suitable to bind the particles of titanium dioxide to the fabric and to its fibers.

The aqueous composition may be applied to the fabric according to techniques that are known per se in the art. For example, according to embodiments, the composition may be provided to the fabric by impregnation, e.g., by immersion of the fabric in a bath containing the composition. According to embodiments, the composition is provided to the fabric by padding.

Subsequently, the fabric provided with the aqueous composition is heated.

According to embodiments, step c) comprises a step of heating the fabric at a first temperature to dry it, and then of heating the fabric at a second temperature suitable to cure the binder polymer on the fabric, i.e. to cross-link it, wherein the second temperature may be higher than the first temperature.

Advantageously, the process of the invention can be carried out, according to embodiments, as a continuous process. For example, the process of the invention can be carried out as a padding process. Padding is a technique that is per se known in the art in the field of textiles. In general, padding process comprises a step of impregnating the fabric with an aqueous composition; the impregnated fabric is passed between at least two rollers, so that the impregnated fabric is pressed by the two rollers, and exceeding composition is removed. Subsequently, the fabric may be dried and optionally cured.

For example, a fabric may be impregnated with the aqueous composition by padding, preferably at a temperature in the range of from 10°C to 50°C, preferably from 20°C to 30°C. The pH of the aqueous composition is, preferably, in the range from 4 to 6, more preferably from 4,5 to 5,5. Subsequently, the fabric impregnated with the aqueous composition may be dried and possibly cured, so that the binder polymer may be cross-linked.

According to an aspect, the process of the invention allows to obtain a fabric wherein the titanium dioxide adheres to yarns and fibers of the fabric. In particular, it has been observed that the process of the invention provides for a fabric wherein titanium dioxide and the binder are placed between the yarns of the fabric, e.g. at the cross-points between the weft and warp yarns of a woven fabric, thus providing increased covering power and a reduction of transparency, with respect to the untreated fabric. For example, in a fabric obtainable according to the invention, titanium dioxide and the binder are also located in the spaces defined by two adjacent warp yarns and two adjacent weft yarns that float over or under said warp yarns, thus providing for a reduction of transparency, with respect to the untreated fabric.

According to embodiments, the fabric provided in step a) of the process of the invention is stretched in at least one direction (e.g., at least in weft direction or at least in warp direction), so that the fabric is stretched during the treatment with the aqueous composition according to step b) of the process of the invention, and preferably also during heating step c).

For example, the fabric may be stretched during padding, heating, and curing step.

It has been observed that when the fabric provided in step a) of the process of the invention is stretched, it is stretched during the treatment with the aqueous composition and preferably also during heating and curing steps, the space between the yarns (e.g., between the warp yarns and/or the weft yarns) increases, so that the composition can be provided between the yarns of the fabric in a particularly effective way. It has been observed that, when the fabric is stretched during the process of the invention, a greater amount of titanium dioxide and binder can be provided between the yarns of the fabric, with respect to the same fabric when it is not stretched during treatment.

According to embodiments, the fabric provided in step a) of the process of the invention is stretched between 0,5% and 75%, preferably between 0,5% and 60%, more preferably between 0,5% and 50%, with respect to the initial dimension of the fabric, in at least one direction (e.g., at least in weft direction) so that the fabric is stretched during the treatment with the aqueous composition according to step b) of the process of the invention, and preferably also during heating step c).

When, for example, the fabric have high elongation at break, such as, e.g., fabrics made from or including elastomeric yarns or fibers, the fabric may be stretched, according to embodiments, between 1% and 75%, preferably between 5% and 60%, more preferably between 10% and 50%, with respect to the initial dimension of the fabric. According to embodiments, the fabric may be stretched at least in weft direction.

When, for example, the fabric have low elongation at break, such as, e.g., fabrics essentially made of natural yarns or fibers, according to embodiments, the fabric may be stretched between 0,5% and 5%, preferably between 0,75% and 5%, more preferably between 1% and 5%, with respect to the initial dimension (e.g., width) of the fabric. According to embodiments, the fabric may be stretched at least in weft direction.

Advantageously, the drying and curing of the fabric provided with the composition, allows to obtain a particularly effective and durable binding of the titanium dioxide to the fabric. This is particularly true when the binder is a crosslinkable binder.

According to embodiments, the crosslinkable binder may be a self-crosslinkable binder. According to embodiments, the crosslinkable binder may be a compound that can be crosslinked using one or more crosslinking agents. Suitable crosslinking agents may be, for example, crosslinking agents including two or more double bonds.

For example, suitable self-crosslinkable binders may be selected from acrylic polymers, acrylic copolymers and acrylic derivatives; for example, suitable binders that can be crosslinked using a crosslinking agent are polyurethanes, which can be crosslinked using, for example, isocyanate.

According to embodiments, when the binder is a crosslinkable binder, a particularly strong binding of the titanium dioxide to the fabric may be obtained.

According to embodiments, the binder, preferably the crosslinkable binder, has a glass transition temperature (Tg) in the range from -30°C to 0°C, preferably from -25°C to -5°C, more preferably from -20°C to -8°C. Advantageously, when the binder, particularly if cross-linkable has glass transition temperature in the above mentioned ranges, a particularly soft treated fabric may be obtained.

Glass transition temperature (Tg) can be measured according to ASTM E1356.

According to embodiments, the binder has a Shore A hardness that is ≤ 30° Shore A, preferably in the range from 5° Shore A to 25° Shore A, more preferably in the range from 10° Shore A to 20° Shore A.

Shore A hardness can be measured according to ASTM D2240.

Binders that are suitable to be used according to the present invention have having glass transition temperature (Tg) and/or hardness in the above mentioned ranges.

As above mentioned, since the binder has glass transition temperature (Tg) and/or Shore A hardness in the above mentioned ranges, it is possible to include titanium dioxide in the binder to obtain a particularly soft and opaque fabric. In particular, it is possible to improve opacity of the fabric without jeopardizing the fabric hand feel.

According to embodiments, the binder may be selected from the group consisting of acrylic polymers, acrylic copolymers and acrylic derivatives, such as vinyl acrylate, styrene acrylate, butadiene acrylonitrile, carboxylated butadiene acrylonitrile; resins; polyurethanes and derivatives thereof, such as polyether polyurethane, polyester polyurethane, polycarbonate polyurethane, polyester polyether polyurethane, polyether polycarbonate polyurethane, polyester polycarbonate polyurethane; blocked isocyanates; poly-isocyanates; and mixtures thereof. According to preferred embodiments, the binder may be selected from the group consisting of butadiene acrylic copolymer, styrene acrylic copolymer, vinyl acrylate, styrene acrylate, butadiene acrylonitrile, carboxylated butadiene acrylonitrile, polyether polyurethane, polyester polyurethane, polycarbonate polyurethane, polyester polyether polyurethane, polyether polycarbonate polyurethane, polyester polycarbonate polyurethane, and mixtures thereof.

For example, the currently commercially available product "ORGAL^{®} ES 61" (Organik kimya), and the commercially available product "HELIZARIN BINDER TOW' (Archroma), are suitable to be used in the composition, according to the invention as a binder.

For example, the currently commercially available product EDOLAN SN (Tanatex Chemicals), which is an aliphatic polyether based polyurethane, is suitable to be used in the composition of the invention, in combination with a crosslinking agent.

As above mentioned, suitable crosslinking agents may be, for example, crosslinking agents including two or more double bonds. For example, the current commercially available product EDOLAN XCIB (Tanatex Chemicals) is suitable to be used as crosslinking agent when EDOLAN SN is used. Advantageously, the binder contributes to the adhesion of titanium dioxide to the fabric.

Advantageously, the present invention allows for the production of a treated fabric which can withstand several home washes. In other words, the present invention allows for the production of a treated fabric which can be home washed several times, while maintaining substantially the same opacity and whiteness characteristics. In particular, it has been observed that, opacity and whiteness characteristics of a fabric treated according to the invention result to be substantially unaltered even after 15 home washings.

According to embodiments, the fabric may be included into a garment, e.g., tailored into a garment, before said step b). In this case, for example, the aqueous composition comprising titanium dioxide and a binder may be provided to the garment by impregnation (e.g., by dipping). Subsequently, the garment may be heat to dry and fix the composition onto the garment.

According to embodiments, the amount of the titanium dioxide in the aqueous composition is in the range from 0,5% to 40% by weight of the composition, preferably in the range from 5% to 30% by weight, more preferably in the range from 10% to 20% by weight.

According to embodiments, titanium dioxide has average particle size in the range from 0,25 µm to 4 µm, preferably from 0,4 µm to 3 µm, more preferably from 0,5 µm to 2 µm.

According to embodiments, the amount of the binder in the composition is in the range of from 0,5% to 10% by weight of said composition, preferably in the range from 2% to 8% by weight, more preferably in the range from 4% to 6% by weight.

According to embodiments, the amount of the binder in the aqueous composition is lower than the amount of the titanium dioxide in the aqueous composition. In this case, advantageously, a white treated fabric having a particularly pleasant appearance and touch can be obtained.

According to embodiments, the composition may further comprise at least one brightening agent. Advantageously, when the aqueous composition includes a brightening agent, a treated fabric having a particularly bright white color can be obtained.

According to embodiments, the brightening agent is preferably stilbene or a stilbene derivative, more preferably a triazine stilbene disulphonic acid, or a derivative thereof. As an example of brightening agent, the currently commercially available product "BLANKOPHOR^{®} B SUN" (Tanatex Chemicals B.V.), is suitable to be used in the composition, according to the invention.

According to embodiments, the amount of the brightening agent in the composition is in the range of from 0,5% to 10% by weight, preferably from 1% to 8% by weight, more preferably from 2% to 5% by weight.

According to embodiments, the aqueous composition may further comprise at least one dispersing agent. As used herein, the term "dispersing agent" refers to an agent suitable to be included into a dispersion, e.g. an aqueous composition, in order to improve the separation of particles in the dispersion, and to prevent settling or clumping.

According to embodiments, the amount of the dispersing agent is in the range of from 0,01% to 2% by weight of the composition, preferably from 0.1% to 1% by weight, more preferably from 0,4% to 0,6% by weight.

According to embodiments, the dispersing agent is selected from polyacrylates, and preferably is an acrylic copolymer. As example of dispersing agents, currently commercially available products "DEKOL^{®} SN 100" (BASF) and "SANYON DQ", are suitable to be used in the composition, according to the invention.

It has been observed that, when the aqueous composition includes a dispersing agent, the distribution of the titanium dioxide on the fabric is particularly homogeneous.

According to embodiments, the aqueous composition may further comprise at least one stabilizing agent. As used herein, the term "stabilizing agent" refers to an agent that substantially prevents the physical and/or chemical alteration of a composition comprising it. Stabilizing agents are known and may be also useful as foam suppressants and/or in the prevention of formation of polymeric films on padding rollers.

According to embodiments, the amount of the stabilizing agent is in the range of from 0,01% to 2% by weight of the composition, preferably from 0.1% to 1% by weight, more preferably from 0,2% to 0,5% by weight.

According to embodiments, the stabilizing agent is an alkoxylate compound or a mixture of alkoxylates. As examples of stabilizing agents, currently commercially available products "VITEXOL PFA" (BASF) and "HELIZARIN COMP. PFA", are suitable to be used in the composition, according to the invention.

According to embodiments, the aqueous composition may further comprise at least one wetting agent. According to embodiments, the amount of the wetting agent is in the range of from 0,01% to 2% by weight of the composition, preferably from 0.1% to 1% by weight, more preferably from 0,2% to 0,4% by weight.

According to embodiments, the wetting agent is a nonionic wetting agent, preferably selected from the group consisting of sulphonate and phosphonate nonionic wetting agents. As an example of wetting agent, the currently commercially available product "COTTOCLARIN TR CT" (BRP Kimya), is suitable to be used in the composition, according to the invention.

According to embodiments, the aqueous composition may further comprise at least one mineral filler different from titanium dioxide. According to embodiments, the amount of the mineral filler is in the range of from 0,1% to 20% by weight of the composition, preferably from 0.5% to 10% by weight, more preferably from 1% to 5% by weight. According to embodiments, the mineral filler may be selected from calcium carbonate, calcium sulfate, kaolin, talc and mixtures thereof.

The process of the invention may be performed using any kind of fabrics. According to embodiments, the fabric is a woven fabric, preferably a twill fabric, and more preferably a denim fabric.

According to embodiments, the fabric may include natural fibres, regenerated fibres, synthetic fibres and mixtures thereof.

According to embodiments, the fabric may include natural yarns and/or regenerated yarns and/or synthetic yarn and/or mixed yarns. In the present description, natural yarns are yarns that include natural fibers, which may be selected from cotton, wool, flax, kenaf, ramie, hemp, linen and mixtures thereof.

In the present description, regenerated yarns are yarns that include regenerated fibers, which may be selected from, for example, viscose, modal, tencel and mixtures thereof.

In the present description, synthetic yarns are yarns that include synthetic fibers, which may be selected from polyester, nylon, polyurethane, spandex (elastane), acrylic, modacrylic, acetate, polyolefin, vinyl and mixtures thereof. In the present description, mixed yarns are yarns that include at least two from natural (e.g., cotton), regenerated and synthetic fibers.

As above mentioned, according to embodiments, step c) of the process of the invention may comprise a step of heating the fabric, provided with the aqueous composition including titanium dioxide and at least one binder, at a first temperature to dry the fabric and then at a second temperature to cure the fabric, i.e. to cross-link the binder applied on the fabric.

According to embodiments, the first temperature ranges from 90°C to 200°C, preferably from 100°C to 160°C, more preferably from 110°C to 150°C. According to embodiments, the second temperature ranges from 150°C to 200°C, preferably from 160°C to 180°C. As above mentioned, according to embodiments, said second temperature is higher than said first temperature. Advantageously, the process according to the invention is particularly fast and easy to be carried out. For example, according to embodiments, step b) of treating the fabric with the aqueous composition comprising titanium dioxide and a binder may have a duration in the range of from 0,1 s to 60 s, preferably 0,5 s to 30 s, more preferably from 1 s to 10 s.

For example, according to embodiments, the step of curing the dry fabric may have a duration in the range of from 15 s to 90 s, preferably from 30 s to 60 s.

Another object of the present invention is a fabric as obtainable through the process according to the invention, i.e. a fabric treated according to the process to increase its opacity.

As above mentioned, it has been observed that in a fabric obtainable according to the invention the titanium dioxide adheres to yarns and fibers of the fabric. It has been also observed that, in a fabric obtainable according to the invention, titanium dioxide also is located between the yarns of the fabric, e.g. at the cross-points between the weft and warp yarns of a woven fabric, thus providing for a reduction of transparency, i.e., an increase of the covering power, with respect to the untreated fabric.

For example, in a fabric obtainable according to the invention, titanium dioxide and the binder are also located in the spaces defined by two adjacent warp yarns and two adjacent weft yarns that float over or under said warp yarns.

According to embodiments, the fabric is a woven fabric comprising weft and warp yarns woven together, and wherein at least part of said titanium dioxide is located at the cross-points between said weft and warp yarns, i.e. the binder including the titanium dioxide is also retained in the points where a warp and a weft yarns cross, and in the spaces defined by two adjacent warp yarns and two adjacent weft yarns that float over or under said warp yarns. The presence of titanium dioxide in these locations greatly increases opacity (or covering power) without making use of low Ne yarns (i.e. high linear density yarns). According to embodiments, the fabric may be twill fabric, preferably a denim fabric.

It has been observed that the relative amount of titanium dioxide disposed between the yarns of the fabric, e.g., between warp yarns and weft yarns, varies according to the structure of the fabric and/or according to the stretching of the fabric during the process of the invention. For example, when the warp density increases, the relative amount of titanium dioxide and binder between the warp yarns reduces.

For example, when the fabric is stretched during the process of the invention, the relative amount of titanium dioxide and binder between the warp yarns of the fabric increases, with respect to the same fabric when it is less stretched or not stretched during the process.

With the wording "treated fabric", "final fabric" it is made reference to a fabric as obtained by the invention process, namely to a fabric used in a garment. The following features and characteristics of the fabric are thus referring to such dry, final, treated fabric as can be found in a garment.

According to embodiments, in the treated fabric the titanium dioxide has average particle size ranging from 0,25 µm to 4 µm, preferably from 0,4 µm to 3 µm, more preferably from 0,5 µm to 2 µm.

According to embodiments, in the final, treated, fabric, the amount of titanium dioxide is in the range of from 3% to 10% by weight of the total weight of the treated fabric, preferably from 6% to 8% by weight of the total weight of the treated fabric, i.e., the treated, dry, fabric.

According to embodiments, the amount of the titanium dioxide in the aqueous composition may be selected in order to obtain a final treated fabric wherein the amount of titanium dioxide is in the range of from 3% to 10% by weight of the total weight of the fabric, preferably from 6% to 8% by weight of the total weight of the fabric.

According to embodiments, in the treated final fabric, e.g. the fabric included in a garment, the amount of the binder is in the range from 0,5% to 4% by weight of the total weight of the treated fabric, preferably from 2% to 3,5% by weight of the total weight of the treated fabric.

According to embodiments, the amount of the binder in the aqueous composition may be selected in order to obtain a treated fabric wherein the amount of the binder is in the range from 0,5% to 4% by weight of the total weight of the fabric, preferably from 2% to 3,5% by weight of the total weight of the fabric.

According to embodiments, the amount of the binder in the fabric is lower than the amount of the titanium dioxide in the fabric. In this case, as above discussed, a white treated fabric having a particularly pleasant appearance and touch can be advantageously obtained. For example, the treated fabric of the invention may comprise an amount of titanium dioxide in the range of from 5% to 10%, preferably from 6% to 8%, by weight of the total weight of the treated fabric, and an amount of binder in the range of from 1% to 5%, preferably from 2% to 4%, by weight of the total weight of the treated fabric.

Advantageously, the treated final fabric of the invention is resistant to washing. In particular, even after several home washings, the opacity, as well as the whiteness, of the fabric is not substantially affected or reduced. Opacity and whiteness may be measured according to known methods, for example by using spectrophotometric techniques.

As used herein, the term "opacity" refers to covering power of the fabric (i.e., to the quality of a textile of being difficult to see through). For example, the higher is the opacity of a fabric, the more is difficult to see through it. In other words, the higher is the opacity of a fabric, i.e., the more a fabric is opaque, the better the fabric prevents what is under the fabric to be revealed through the fabric.

According to embodiments, the binder has a glass transition temperature (Tg) in the range from -30°C to 0°C, preferably from -25°C to -5°C, more preferably from -20°C to -8°C. In this case, advantageously, a particularly soft treated fabric may be obtained.

Glass transition temperature (Tg) can be measured according to ASTM E1356.

According to embodiments, the binder has a Shore A hardness ≤ 30° Shore A, preferably in the range from 5° Shore A to 25° Shore A, more preferably in the range from 10° Shore A to 20° Shore A.

Shore A hardness can be measured according to ASTM D2240.

As above mentioned, since the binder has glass transition temperature (Tg) and/or Shore A hardness in the above mentioned ranges, it is possible to obtain a particularly soft opaque fabric.

According to embodiments, the fabric of the invention, in addition to titanium dioxide and at least one binder may optionally include one or more brightening agents and/or one or more dispersing agent and/or one or more stabilizing agent and/or one or more wetting agent.

According to embodiments, the final treated fabric may comprise a brightening agent in an amount in the range from 0,5% to 3%, preferably 1% to 2% by weight of the total weight of the treated fabric. According to embodiments, the amount of the brightening agent in the aqueous composition may be selected in order to obtain a fabric wherein the amount of the brightening agent is in the range from 0,5% to 3%, preferably 1% to 2% by weight of the total weight of the treated fabric.

According to embodiments, the fabric may comprise a dispersing agent in an amount in the range from 0,1% to 1%, preferably 0,2% to 0,5% by weight of the total weight of the treated fabric. According to embodiments, the amount of the dispersing agent in the aqueous composition may be selected in order to obtain a fabric wherein the amount of the dispersing agent is in the range from 0,1% to 1%, preferably 0,2% to 0,5% by weight of the total weight of the treated fabric.

According to embodiments, the invention fabric may comprise a stabilizing agent in an amount in the range from 0,1% to 0,5%, preferably from 0,2% to 0,4%, by weight of the total weight of the treated fabric. According to embodiments, the amount of the stabilizing agent in the aqueous composition may be selected in order to obtain a treated fabric wherein the amount of the stabilizing agent is in the range from 0,1% to 0,5%, preferably from 0,2% to 0,4%, by weight of the total weight of the treated fabric.

According to embodiments, the invention fabric may comprise a wetting agent in an amount in the range of from 0,05% to 0,5% by weight, preferably 0,1% to 0,4% by weight of the total weight of the fabric. According to embodiments, the amount of the wetting agent in the aqueous composition may be selected in order to obtain a treated fabric wherein the amount of the wetting agent is in the range of from 0,05% to 0,5% by weight, preferably 0,1% to 0,4% by weight of the total weight of the fabric.

The composition on the invention fabric can be analyzed according to known methods, in order to determine the amount of the components included in said dried and cured composition. For example, titanium dioxide can be extracted from the treated fabric, isolated and separated according to known methods, and characterized according to ASTM D1394 - Test for Chemical Analysis of White Titanium Pigments.

According to an aspect of the present invention, the fabric of the invention is suitable to be tailored into a garment. A further object of the invention is a garment comprising a fabric according to the invention. Advantageously, the skin of the user is not (partly) visible through the fabric treated according to the invention. Similarly, any underwear of the user worn under a garment according to the invention in not visible through the said garment.

A further object of the present invention is an aqueous composition for treatment of textiles, namely of a fabric, preferably of a woven fabric, comprising:
- titanium dioxide in an amount in the range from 5 to 500 g/L, preferably in the range from 50 to 400 g/L, more preferably in the range from 75 to 300 g/L, even more preferably in the range of from 90 to 200 g/L; and
- at least one binder, preferably a cross-linkable binder, in an amount in the range from 1 to 100 g/L, preferably in the range from 10 to 80 g/L, more preferably in the range from 30 to 70 g/L, even more preferably in the range from 35 to 60 g/L;
wherein said binder has a glass transition temperature (Tg) in the range from -30°C to 0°C, wherein glass transition temperature (Tg) is measured according to ASTM E1356, and/or a Shore A hardness that is ≤ 30° Shore A, wherein Shore A hardness is measured according to ASTM D2240.

According to embodiments, the aqueous composition may comprise:
- titanium dioxide in an amount in the range from 0,5% to 40% by weight of said composition, preferably in the range from 5% to 30% by weight, more preferably in the range from 10% to 20% by weight; and
- at least one binder, preferably crosslinkable binder, in an amount in the range from 0,5% to 10% by weight of said composition, preferably in the range from 2% to 8% by weight, more preferably in the range from 4% to 6% by weight.

The aqueous composition that is object of the invention is suitable to be used in the process of the invention. Therefore, the features of the aqueous composition disclosed above with reference to the composition in the process of the invention, are intended to apply to the composition per se, and vice versa, i.e., the feature herein disclosed with reference to the aqueous composition per se are intended to apply to the composition in the process of the invention.

Advantageously, the aqueous composition may be produced through known methods. For example, it may be produced by mixing the different components. According to embodiments, the components may be provided and admixed together to obtain the aqueous composition. According to embodiments, two or more components may be provided sequentially during the mixing.

According to embodiments, the aqueous composition may have a pH in the range of from 4 to 6, preferably from 4,5 to 5. According to embodiments, the aqueous composition further comprises at least one brightening agent in an amount in the range from 0,5% to 10% by weight of said composition, preferably from 1% to 8% by weight, more preferably from 2% to 5% by weight.

According to embodiments, the aqueous composition comprises:
- from 5 to 500 g/L of titanium dioxide,
- from 1 to 100 g/L of at least one binder.

According to embodiments, the concentration of titanium dioxide in the aqueous composition may be in the range of from 50 to 400 g/L, preferably from 75 to 300 g/L, more preferably from 90 to 200 g/L.

According to embodiments, the concentration of the binder in the aqueous composition may be in the range of from 10 to 80 g/L, preferably 30 to 70 g/L, preferably from 35 to 60 g/L.

According to embodiments, the aqueous composition may further comprise one or more brightening agents. According to embodiments, the concentration of the brightening agent in the aqueous composition may be in the range of from 5 to 40 g/L, preferably from 10 to 35 g/L, more preferably from 15 to 30 g/L.

According to embodiments, the aqueous composition may further comprise one or more dispersing agent. According to embodiments, the concentration of the dispersing agent in the aqueous composition may be in the range of from 1 to 20 g/L, preferably from 2.5 to 10 g/L, more preferably from 4 to 6 g/L.

According to embodiments, the aqueous composition may further comprise one or more stabilizing agent. According to embodiments, the concentration of the stabilizing agent in the aqueous composition is in the range of from 1 to 10 g/L, preferably from 2 to 6 g/L, more preferably from 3 to 5 g/L.

According to embodiments, the aqueous composition may further comprise one or more wetting agents. According to embodiments, the concentration of the wetting agent in the aqueous composition is in the range of from 0,5 g/L to 10 g/L, preferably from 1 to 5 g/L, more preferably from 2 to 4 g/L.

According to embodiments, the aqueous composition may further comprise one or more mineral filler different from titanium dioxide. According to embodiments, the concentration of the mineral filler different from titanium dioxide in the aqueous composition is in the range of from 10 to 100 g/L, preferably from 10 to 50 g/L, of at least one mineral filler. According to embodiments, the mineral filler is selected from the group consisting of calcium carbonate, calcium sulfate, kaolin, talc and mixtures thereof.

Also object of the present invention is the use of a composition according to the invention in the process according to invention.

Advantageously, the present invention allows to obtain a white fabric having high opacity in easier, faster and cheaper way, with respect to the processes that are known in the art.

### Experimental Section

### Example 1 - Compositions

Example 1 refers to different embodiments of the aqueous composition of the invention.

In all the exemplary composition, the final volume of the aqueous composition is 1 L.

### Composition 1:

| | |
|---|---|
| Titanium dioxide | 100 g/L |
| ORGAL^{®} ES 61 | 40 g/L |
| Water | up to a final volume of 1 L |

### Composition 2:

| | |
|---|---|
| Titanium dioxide | 100 g/L |
| ORGAL^{®} ES 61 | 40 g/L |
| SANYON DQ | 5 g/L |
| HELIZARIN COMP. PFA | 4 g/L |
| BLANKOPHOR^{®} B SUN | 20 g/L |
| COTTOCLARIN TR CT | 3 g/L |
| Water | up to a final volume of 1 L |

### Composition 3:

| | |
|---|---|
| Titanium dioxide | 100 g/L |
| ORGAL^{®} ES 61 | 40 g/L |
| SANYON DQ | 5 g/L |
| HELIZARIN COMP. PFA | 4 g/L |
| COTTOCLARIN TR CT | 3 g/L |
| Water | up to a final volume of 1 L |

In the above mentioned compositions 1-3, ORGAL^{®} ES 61 (styrene acrylic copolymer, having a Tg of -12°C) was the binder, SANYON DQ was the dispersing agent, HELIZARIN COMP. PFA was the stabilizing agent, BLANKOPHOR^{®} B SUN was the brightening agent and COTTOCLARIN TR CT was the wetting agent.

### Composition 4:

| | |
|---|---|
| Titanium Dioxide: | 100 g/l |
| HELIZARIN BINDER TOW: | 46 g/l |
| SANYON DQ: | 5 g/l |
| HELIZARIN COMP. PFA: | 4 g/l |
| COTTOCLARIN TR CT: | 3 g/l |
| Water: | up to a final volume of 1L |

### Composition 5:

| | |
|---|---|
| Titanium Dioxide: | 100 g/l |
| HELIZARIN BINDER TOW: | 46 g/l |
| SANYON DQ: | 5 g/l |
| HELIZARIN COMP. PFA: | 4 g/l |
| BLANKOPHOR^{®} B SUN: | 20 g/l |
| COTTOCLARIN TR CT: | 3 g/l |
| Water: | up to a final volume of 1L |

In the above mentioned compositions 4-5, HELIZARIN BINDER TOW (acrylic copolymer, having a Tg of -18°C) was the binder, SANYON DQ was the dispersing agent, HELIZARIN COMP. PFA was the stabilizing agent, BLANKOPHOR^{®} B SUN was the brightening agent and COTTOCLARIN TR CT was the wetting agent.

### Composition 6:

| | |
|---|---|
| Titanium Dioxide: | 100 g/l |
| EDOLAN SN: | 30 g/l |
| EDOLAN XCIB: | 5 g/l |
| SANYON DQ: | 5 g/l |
| HELIZARIN COMP. PFA: | 4 g/l |
| COTTOCLARIN TR CT: | 3 g/l |
| Water: | up to a final volume of 1L |

### Composition 7:

| | |
|---|---|
| Titanium Dioxide: | 100 g/l |
| EDOLAN SN: | 30 G/L |
| EDOLAN XCIB: | 5 G/L |
| SANYON DQ: | 5 G/L |
| HELIZARIN COMP. PFA: | 4 G/L |
| BLANKOPHOR^{®} B-SUN: | 20 G/L |
| COTTOCLARIN TR CT: | 3 g/l |
| Water: | up to a final volume of 1L |

In the above mentioned compositions 6-7, EDOLAN SN (aliphatic polyether based polyurethane) was the binder, EDOLAN XCIB was the crosslinking agent, SANYON DQ was the dispersing agent, HELIZARIN COMP. PFA was the stabilizing agent, BLANKOPHOR^{®} B SUN was the brightening agent and COTTOCLARIN TR CT was the wetting agent. The Shore A hardness of the binder EDOLAN SN crosslinked with the crosslinking agent EDOLAN XCIB is 20° Shore A.

All the compositions 1-7 above mentioned may be produced by mixing the components and stirring to obtain a homogeneous mixture (for example, stirring for about 30 minutes).

### Example 2 - production of treated fabrics

### Treated fabric 1

A cotton woven fabric was treated with the "Composition 1" according to Example 1.

The aqueous composition was applied by padding.

The fabric was dried 150 °C and cured at 180 °C for 45 seconds.

The treated fabric obtained was provided with:

| | |
|---|---|
| Titanium dioxide | about 7% by weight |
| Binder | about 2.8% by weight |

The amounts are expressed as percentage by weight of the total weight of the treated fabric.

### Treated fabric 2

A cotton woven fabric was treated with the "Composition 3" according to Example 1.

The aqueous composition was applied by padding.

The fabric was dried 150 °C and cured at 180 °C for 45 seconds.

The treated fabric obtained was provided with:

| | |
|---|---|
| Titanium dioxide | about 7% by weight |
| Binder | about 2.8% by weight |
| Dispersing agent | about 0.35% by weight |
| Stabilizing agent | about 0.28% by weight |
| Wetting agent | about 0.2% by weight |

The amounts are expressed as percentage by weight of the total weight of the treated fabric.

### Treated fabric 3

A cotton woven fabric was treated with the "Composition 4" according to Example 1.

The aqueous composition was applied by padding.

The fabric was dried 150 °C and cured at 180 °C for 45 seconds.

The treated fabric obtained was provided with:

| | |
|---|---|
| Titanium dioxide | about 7% by weight |
| Binder | about 3.22% by weight |
| Dispersing agent | about 0.35% by weight |
| Stabilizing agent | about 0.28% by weight |
| Wetting agent | about 0.2% by weight |

The amounts are expressed as percentage by weight of the total weight of the treated fabric.

### Treated fabric 4

A cotton woven fabric was treated with the "Composition 6" according to Example 1.

The aqueous composition was applied by padding.

The fabric was dried 150 °C and cured at 180 °C for 45 seconds.

The treated fabric obtained was provided with:

| | |
|---|---|
| Titanium dioxide | about 7% by weight |
| Binder | about 2.1% by weight |
| Crosslinking agent | about 0.35% by weight |
| Dispersing agent | about 0.35% by weight |
| Stabilizing agent | about 0.28% by weight |
| Wetting agent | about 0.2% by weight |

The amounts are expressed as percentage by weight of the total weight of the treated fabric.

### Example 3 - evaluation of opacity and CMC DE (color difference) of exemplary treated fabrics

Opacity and CMC DE (color difference) of three samples of a fabric before and after the process of the invention were measured.

In particular, the fabric was treated to obtain the "Treated fabric 1", the "Treated fabric 3" and the "Treated fabric 4" according to Example 2.

Opacity and CMC DE (color difference) were measured spectrophotometrically, according to methods which are known per se, using white and black background cards, by Datacolor 600 spectrophotometer.

Opacity of fabrics was measured, on paper backing, as the ratio expressed as a percentage, of the single-sheet luminous reflectance factor, R₀, to the intrinsic luminous reflectance factor, R∞, of the same sample, according to the formula:$Opacity = 100 x {R}_{0} /R ∞$

The single-sheet luminous reflectance factor, "R₀" is defined as the luminous reflectance factor of a single sheet of fabric with a black cavity as backing.

The intrinsic luminous reflectance factor, "R_{∞}" is defined as the luminous reflectance factor of a layer or pad of fabric which have a thickness such that a further increase in the thickness of the layer or pad results in no change in the measured reflectance factor. In this case, the single sheet of fabric is a single fabric when it is not folded, so that the thickness of the layer or pad above mention corresponds to the thickness of a single fabric. The thickness of the layer or pad may be increased, for example, by folding the fabric so that two or more portion of the same fabric are the superimposed in order to increase the thickness of the layer or pad to be analyzed, up to a thickness which provides for a reflectance factor value which does not changes if the thickness of the layer or pad is further increased.

"CMC DE" is the difference between a sample color and a reference color. CMC DE was measured using white and black background cards, by Datacolor 600 spectrophotometer. Firstly, a fabric was placed over white background and reflectance was measured as reference, using Datacolor 600 spectrophotometer. Then, the same fabric was placed over black background and reflectance was measured as sample, using Datacolor 600. CMC DE (i.e., color difference) between the fabric over white background and the fabric over black background is determined spectrophotometrically according to known methods. The smaller the CMC DE value is, the more the fabric is opaque. In other words, the more a fabric is opaque, the smaller the color difference between over white and over black is.

The following results were obtained:
Untreated fabric
   CMC DE : 3,17
   Opacity : 87%
Treated fabric 1 according to Example 2
   CMC DE : 1,84
   Opacity : 95%
   Treated fabric 3 according to Example 2
   CMC DE : 1,90
   Opacity : 95,8%
   Treated fabric 4 according to Example 2
   CMC DE : 1,91
   Opacity : 95,32%

As can be observed, in the case of "Treated fabric 1", the process of the invention allowed an increase in the opacity of the fabric of about 8% with respect to the untreated fabric. Also, the process of the invention allowed a reduction of the CMC DE (i.e., the color difference) of about 42% with respect to the untreated fabric.

In the case of "Treated fabric 3", the process of the invention allowed an increase in the opacity of the fabric of about 8,8% with respect to the untreated fabric. Also, the process of the invention allowed a reduction of the CMC DE (i.e., the color difference) of about 40% with respect to the untreated fabric.

In the case of "Treated fabric 4", the process of the invention allowed an increase in the opacity of the fabric of about 8,3% with respect to the untreated fabric. Also, the process of the invention allowed a reduction of the CMC DE (i.e., the color difference) of about 39,7% with respect to the untreated fabric.

The results obtainable through the process of the invention can also be observed in the attached Figures, which show a sample fabric before and after the process of the invention, at different magnifications.

In particular, Figure 1A and Figure 1B are photographs showing a sample fabric before (Figure 1A) and after (Figure 1B) the process of the invention.

Figure 2A and Figure 2B are photographs taken at magnification of 10X and Figure 3A and Figure 3B are photographs taken at magnification of 60X.

As can be observed, for example from Figure 1A and 1B, and Figure 2A and 2B, the treated fabric of the invention has an improved opacity and whiteness with respect to the untreated fabric.

In Figure 3B particles of titanium dioxide between the fibers and yarns of the treated fabric can be observed. Such particles cannot be observed in Figure 3A, which shows an untreated fabric. Figure 3A and Figure 3B show that the present invention is, advantageously, effective in providing titanium dioxide to fabrics.

## Claims

1. A process for producing a fabric, comprising the step of:
a) Providing at least a fabric,
b) treating at least part of said fabric with an aqueous composition comprising titanium dioxide and at least a binder, preferably a crosslinkable binder,
c) heating the fabric obtained in step b);
wherein said binder has a glass transition temperature (Tg) in the range from -30°C to 0°C, wherein glass transition temperature (Tg) is measured according to ASTM E1356, and/or a Shore A hardness that is ≤ 30° Shore A, wherein Shore A hardness is measured according to ASTM D2240.

2. The process according to claim 1, wherein said step c) comprises heating said fabric at a first temperature to dry said fabric and then heating said fabric at a second temperature to cross-link said binder on said fabric, said second temperature preferably being higher than said first temperature.

3. The process according to claim 1 or 2, wherein said fabric provided in said step a) is stretched in at least one direction, so that the fabric is in a stretched condition during the treatment with the aqueous composition according to step b) of the process of the invention, and preferably also during heating step c).

4. The process according to claim 3, wherein said fabric provided in said step a) is stretched between 0,5% and 75%, preferably between 0,5% and 60%, more preferably between 0,5% and 50%, with respect to the initial dimension of the fabric, at least in weft direction.

5. The process according to any claim 1 to 4, wherein in said step b), said aqueous composition is provided to said fabric by padding.

6. The process according to any previous claim, wherein said binder is selected from the group consisting of acrylic polymers, acrylic copolymers and acrylic derivatives, resins, polyurethanes and polyurethane derivatives, blocked isocyanates, poly-isocyanates, and mixtures thereof, and preferably is selected from the group consisting of butadiene acrylic copolymer, styrene acrylic copolymer, vinyl acrylate, styrene acrylate, butadiene acrylonitrile, carboxylated butadiene acrylonitrile, polyether polyurethane, polyester polyurethane, polycarbonate polyurethane, polyester polyether polyurethane, polyether polycarbonate polyurethane, polyester polycarbonate polyurethane, and mixtures thereof.

7. The process according to any previous claim, wherein said binder, preferably said crosslinkable binder, has a glass transition temperature (Tg) in the range from -25°C to -5°C, preferably from -20°C to -8°C, wherein glass transition temperature (Tg) is measured according to ASTM E1356.

8. The process according to any previous claim, wherein said binder has a Shore A hardness in the range from 5° Shore A to 25° Shore A, preferably in the range from 10° Shore A to 20° Shore A, wherein Shore A hardness is measured according to ASTM D2240.

9. The process according to any previous claim, wherein said fabric is included into a garment before said step b).

10. The process according to any previous claim, wherein said titanium dioxide in said composition is in the range from 5 to 500 g/L, preferably in the range from 50 to 400 g/L, more preferably in the range from 75 to 300 g/L, even more preferably in the range of from 90 to 200 g/L.

11. The process according to any previous claim, wherein said titanium dioxide has average particle size in the range from 0.25 µm to 4 µm, preferably from 0.4 µm to 3 µm, more preferably from 0.5 µm to 2 µm.

12. The process according to any previous claim, wherein said binder in said composition is in the range of from 1 to 100 g/L, preferably in the range from 10 to 80 g/L, more preferably in the range from 30 to 70 g/L, even more preferably in the range from 35 to 60 g/L.

13. The process according to any previous claim, wherein said composition further comprises at least one brightening agent, preferably stilbene or a stilbene derivative, more preferably a triazine stilbene disulphonic acid, or a derivative thereof.

14. The process according to claim 13, wherein the amount of said brightening agent in said composition is in the range of from 5 to 40 g/L, preferably from 10 to 35 g/L, more preferably from 15 to 30 g/L.

15. The process according to any claim 2 to 14, wherein said first temperature is in the range of 90°C to 200°C, preferably of 100°C to 160°C, more preferably of 110°C to 150°C.

16. The process according to any claim 2 to 15, wherein said second temperature is in the range of 150°C to 200°C, preferably of 160° to 180°C.

17. A fabric as obtainable through a process according to any claim 1 to 16.

18. A fabric according to claim 17, wherein said fabric is a woven fabric comprising weft and warp yarns woven together, and wherein at least part of said titanium dioxide and of said binder is located in the spaces defined by two adjacent warp yarns and two adjacent weft yarns that float over or under said warp yarns.

19. A fabric according to claim 18, wherein said fabric is twill fabric, preferably a denim fabric.

20. A fabric according to any claim 17 to 19, wherein the said titanium dioxide has average particle size in the range of 0.25 µm to 4 µm, preferably 0.4 µm to 3 µm, more preferably 0.5 µm to 2 µm.

21. A fabric according to any claim 17 to 20, wherein the amount of said titanium dioxide is in the range from 3% to 10% by weight of the fabric, preferably from 6% to 8% by weight of the total weight of the fabric.

22. A fabric according to any claim 17 to 21, wherein the amount of said binder is in the range from 0.5% to 4% by weight of the fabric, preferably from 2% to 3% by weight of the total weight of said fabric.

23. A garment comprising a fabric according to any claim 17 to 22.

24. An aqueous composition for treating a textile, preferably a fabric, comprising:
• titanium dioxide in an amount in the range from 5 to 500 g/L, preferably in the range from 50 to 400 g/L, more preferably in the range from 75 to 300 g/L, even more preferably in the range of from 90 to 200 g/L; and
• at least one binder, preferably a cross-linkable binder, in an amount in the range from 1 to 100 g/L, preferably in the range from 10 to 80 g/L, more preferably in the range from 30 to 70 g/L, even more preferably in the range from 35 to 60 g/L;
wherein said binder has a glass transition temperature (Tg) in the range from -30°C to 0°C, wherein glass transition temperature (Tg) is measured according to ASTM E1356, and/or a Shore A hardness that is ≤ 30° Shore A wherein Shore A hardness is measured according to ASTM D2240.

25. Composition according to claim 24, further comprising at least one brightening agent in an amount in the range from 5 to 40 g/L, preferably from 10 to 35 g/L, more preferably from 15 to 30 g/L.

26. Use of a composition according to claim 24 or 25 in the process according to any claim 1-16.

## Patentansprüche

1. Ein Verfahren zur Herstellung eines Gewebes, aufweisend die Schritte:
a) Bereitstellen zumindest eines Gewebes,
b) Behandeln von zumindest einem Teil des Gewebes mit einer wässrigen Zusammensetzung, enthaltend Titandioxid und zumindest ein Bindemittel, vorzugsweise ein vernetzbares Bindemittel,
c) Erwärmen des in Schritt b) erhaltenen Gewebes,
wobei das Bindemittel eine Glasübergangstemperatur (Tg) im Bereich von -30°C bis 0°C aufweist, wobei die Glasübergangstemperatur (Tg) gemäß ASTM E1356 gemessen ist, und/oder eine Shore-A-Härte ≤ 30° Shore A ist, wobei die Shore-A-Härte gemäß ASTM D2240 gemessen ist.

2. Das Verfahren gemäß Anspruch 1, wobei der Schritt c) das Erwärmen des Gewebes auf eine erste Temperatur zum Trocknen des Gewebes und dann das Erwärmen des Gewebes auf eine zweite Temperatur zum Vernetzen des Bindemittels auf dem Gewebe aufweist, wobei die zweite Temperatur vorzugsweise höher als die erste Temperatur ist.

3. Das Verfahren gemäß Anspruch 1 oder 2, wobei das in Schritt a) bereitgestellte Gewebe in mindestens eine Richtung gedehnt wird, so dass sich das Gewebe während der Behandlung mit der wässrigen Zusammensetzung gemäß Schritt b) des erfindungsgemäßen Verfahrens und vorzugsweise auch während des Erwärmungsschritts c) in einem gedehnten Zustand befindet.

4. Das Verfahren gemäß Anspruch 3, wobei das in Schritt a) bereitgestellte Gewebe zumindest in Schussrichtung zwischen 0,5 % und 75 %, vorzugsweise zwischen 0,5 % und 60 %, bevorzugter zwischen 0,5 % und 50 %, in Bezug auf die ursprüngliche Abmessung des Gewebes gedehnt wird.

5. Das Verfahren gemäß einem der Ansprüche 1 bis 4, wobei in dem Schritt b) die wässrige Zusammensetzung durch Wattierung auf den Stoff aufgebracht wird.

6. Verfahren nach einem der vorhergehenden Ansprüche, wobei das Bindemittel ausgewählt ist aus der Gruppe, bestehend aus Acrylpolymeren, Acrylcopolymeren und Acrylderivaten, Harzen, Polyurethanen und Polyurethanderivaten, blockierten Isocyanaten, Polyisocyanaten und Mischungen davon, und vorzugsweise ausgewählt ist aus der Gruppe, bestehend aus Butadien-Acryl-Copolymer, Styrol-Acryl-Copolymer, Vinylacrylat, Styrolacrylat, Butadien-Acrylnitril, carboxyliertem Butadien-Acrylnitril, Polyether-Polyurethan, Polyester-Polyurethan, Polycarbonat-Polyurethan, Polyester-Polyether-Polyurethan, Polyether-Polycarbonat-Polyurethan, Polyester-Polycarbonat-Polyurethan und Mischungen davon.

7. Das Verfahren gemäß einem der vorhergehenden Ansprüche, wobei das Bindemittel, vorzugsweise das vernetzbare Bindemittel, eine Glasübergangstemperatur (Tg) im Bereich von -25 °C bis -5 °C, bevorzugter von -20 °C bis -8 °C aufweist, wobei die Glasübergangstemperatur (Tg) gemäß ASTM E1356 gemessen ist.

8. Das Verfahren gemäß einem der vorhergehenden Ansprüche, wobei das Bindemittel eine Shore-A-Härte im Bereich von 5° Shore A bis 25° Shore A, bevorzugter im Bereich von 10° Shore A bis 20° Shore A aufweist, wobei die Shore-A-Härte gemäß ASTM D2240 gemessen ist.

9. Das Verfahren gemäß einem der vorhergehenden Ansprüche, wobei das Gewebe vor dem Schritt b) in ein Kleidungsstück eingearbeitet wird.

10. Das Verfahren gemäß einem der vorhergehenden Ansprüche, wobei der Titandioxidgehalt in der Zusammensetzung im Bereich von 5 bis 500 g/L, vorzugsweise im Bereich von 50 bis 400 g/L, bevorzugter im Bereich von 75 bis 300 g/L, noch bevorzugter im Bereich von 90 bis 200 g/L liegt.

11. Das Verfahren gemäß einem der vorhergehenden Ansprüche, wobei das Titandioxid eine durchschnittliche Partikelgröße im Bereich von 0,25 µm bis 4 µm, vorzugsweise von 0,4 µm bis 3 µm, stärker bevorzugt von 0,5 µm bis 2 µm aufweist.

12. Das Verfahren gemäß einem der vorhergehenden Ansprüche, wobei der Bindemittelgehalt in der Zusammensetzung im Bereich von 1 bis 100 g/L, vorzugsweise im Bereich von 10 bis 80 g/L, bevorzugter im Bereich von 30 bis 70 g/L, noch bevorzugter im Bereich von 35 bis 60 g/L liegt.

13. Das Verfahren gemäß einem der vorhergehenden Ansprüche, wobei die Zusammensetzung außerdem mindestens ein Aufhellmittel, vorzugsweise Stilben oder ein Stilbenderivat, bevorzugter eine Triazin-Stilbendisulfonsäure oder ein Derivat davon, enthält.

14. Das Verfahren gemäß Anspruch 13, wobei die Menge des Aufhellmittels in der Zusammensetzung im Bereich von 5 bis 40 g/L, vorzugsweise von 10 bis 35 g/L, bevorzugter von 15 bis 30 g/L liegt.

15. Das Verfahren gemäß einem der Ansprüche 2 bis 14, wobei die erste Temperatur im Bereich von 90°C bis 200°C, vorzugsweise von 100°C bis 160°C, bevorzugter von 110°C bis 150°C liegt.

16. Das Verfahren gemäß einem der Ansprüche 2 bis 15, wobei die zweite Temperatur im Bereich von 150°C bis 200°C, vorzugsweise von 160°C bis 180°C liegt.

17. Ein Gewebe, erhältlich durch ein Verfahren gemäß einem der Ansprüche 1 bis 16.

18. Ein Gewebe nach Anspruch 17, wobei das Gewebe ein gewebtes Gewebe ist, das aus miteinander verwebten Schuss- und Kettfäden besteht, und wobei sich zumindest ein Teil des Titandioxids und des Bindemittels in den Zwischenräumen befindet, die durch zwei benachbarte Kettfäden und zwei benachbarte Schussfäden definiert sind, die über oder unter den Kettfäden schweben.

19. Ein Gewebe nach Anspruch 18, wobei das Gewebe ein Köpergewebe, vorzugsweise ein Denimgewebe ist.

20. Ein Gewebe nach einem der Ansprüche 17 bis 19, wobei das Titandioxid eine durchschnittliche Partikelgröße im Bereich von 0,25 µm bis 4 µm, vorzugsweise 0,4 µm bis 3 µm, stärker bevorzugt 0,5 µm bis 2 µm aufweist.

21. Ein Gewebe nach einem der Ansprüche 17 bis 20, wobei die Menge des Titandioxids im Bereich von 3 bis 10 Gew.-% des Gewebes, vorzugsweise von 6 bis 8 Gew.-% des Gesamtgewichts des Gewebes liegt.

22. Ein Gewebe nach einem der Ansprüche 17 bis 21, wobei die Menge des Bindemittels im Bereich von 0,5 bis 4 Gew.-% des Gewebes, vorzugsweise von 2 bis 3 Gew.-% des Gesamtgewichts des Gewebes liegt.

23. Ein Kleidungsstück, aufweisend einen Stoff gemäß einem der Ansprüche 17 bis 22.

24. Eine wässrige Zusammensetzung zur Behandlung eines Stoffes, vorzugsweise eines Gewebes, enthaltend:
• Titandioxid in einer Menge im Bereich von 5 bis 500 g/L, vorzugsweise im Bereich von 50 bis 400 g/L, bevorzugter im Bereich von 75 bis 300 g/L, noch bevorzugter im Bereich von 90 bis 200 g/L; und
• mindestens ein Bindemittel, vorzugsweise ein vernetzbares Bindemittel, in einer Menge im Bereich von 1 bis 100 g/L, vorzugsweise im Bereich von 10 bis 80 g/L, bevorzugter im Bereich von 30 bis 70 g/L, noch bevorzugter im Bereich von 35 bis 60 g/L;
wobei das Bindemittel eine Glasübergangstemperatur (Tg) im Bereich von -30°C bis 0°C aufweist, wobei die Glasübergangstemperatur (Tg) gemäß ASTM E1356 gemessen ist, und/oder eine Shore-A-Härte ≤ 30° Shore A ist, wobei die Shore-A-Härte gemäß ASTM D2240 gemessen ist.

25. Zusammensetzung nach Anspruch 24, die außerdem mindestens ein Aufhellungsmittel in einer Menge im Bereich von 5 bis 40 g/L, vorzugsweise von 10 bis 35 g/L, weiter bevorzugt von 15 bis 30 g/L, enthält.

26. Verwendung einer Zusammensetzung gemäß Anspruch 24 oder 25 im Verfahren gemäß einem der Ansprüche 1 bis16.

## Revendications

1. Procédé de fabrication d'un tissu, comprenant l'étape consistant à :
a) Fournir au moins un tissu,
b) traiter au moins une partie dudit tissu avec une composition aqueuse comprenant du dioxyde de titane et au moins un liant, de préférence un liant réticulable,
c) chauffer le tissu obtenu à l'étape b) ;
dans lequel ledit liant a une température de transition vitreuse (Tg) comprise entre-30°C et 0°C, dans lequel la température de transition vitreuse (Tg) est mesurée selon la norme ASTM E1356, et/ou une dureté Shore A ≤ 30° Shore A, dans lequel la dureté Shore A est mesurée selon la norme ASTM D2240.

2. Procédé selon la revendication 1, dans lequel ladite étape c) comprend le chauffage dudit tissu à une première température pour sécher ledit tissu, puis le chauffage dudit tissu à une seconde température pour réticuler ledit liant sur ledit tissu, ladite seconde température étant de préférence supérieure à ladite première température.

3. Procédé selon la revendication 1 ou 2, dans lequel ledit tissu fourni dans ladite étape a) est étiré dans au moins une direction, de sorte que le tissu est dans un état étiré pendant le traitement avec la composition aqueuse selon l'étape b) du procédé de l'invention, et de préférence aussi pendant l'étape c) de chauffage.

4. Procédé selon la revendication 3, dans lequel ledit tissu fourni dans ladite étape a) est étiré entre 0,5 % et 75 %, de préférence entre 0,5 % et 60 %, plus préférentiellement entre 0,5 % et 50 %, par rapport à la dimension initiale du tissu, au moins dans la direction de trame.

5. Procédé selon l'une quelconque des revendications 1 à 4, dans lequel, dans ladite étape b), ladite composition aqueuse est fournie au tissu par rembourrage.

6. Procédé selon l'une quelconque des revendications précédentes, dans lequel ledit liant est choisi dans le groupe constitué des polymères acryliques, les copolymères acryliques et les dérivés acryliques, les résines, les polyuréthanes et les dérivés de polyuréthane, les isocyanates bloqués, les poly-isocyanates, et leurs mélanges, et de préférence est choisi dans le groupe constitué du copolymère acrylique de butadiène, copolymère styrène acrylique, acrylate de vinyle, acrylate de styrène, butadiène acrylonitrile, butadiène acrylonitrile carboxylé, polyéther polyuréthane, polyester polyuréthane, polycarbonate polyuréthane, polyester polyéther polyuréthane, polyéther polycarbonate polyuréthane, polyester polycarbonate polyuréthane, et leurs mélanges.

7. Procédé selon l'une quelconque des revendications précédentes, dans lequel ledit liant, de préférence ledit liant réticulable, a une température de transition vitreuse (Tg) comprise entre -25°C et -5°C, de préférence entre -20°C et -8°C, dans lequel la température de transition vitreuse (Tg) est mesurée selon la norme ASTM E1356.

8. Procédé selon l'une quelconque des revendications précédentes, dans lequel ledit liant a une dureté Shore A comprise entre 5° Shore A et 25° Shore A, de préférence entre 10° Shore A et 20° Shore A, dans lequel la dureté Shore A est mesurée selon la norme ASTM D2240.

9. Procédé selon l'une quelconque des revendications précédentes, dans lequel ledit tissu est inclus dans un vêtement avant ladite étape b).

10. Procédé selon l'une quelconque des revendications précédentes, dans lequel ledit dioxyde de titane dans ladite composition est compris entre 5 et 500 g/L, de préférence entre 50 et 400 g/L, plus préférentiellement entre 75 et 300 g/L, encore plus préférentiellement entre 90 et 200 g/L.

11. Procédé selon l'une quelconque des revendications précédentes, dans lequel ledit dioxyde de titane a une taille moyenne de particules comprise entre 0,25 µm et 4 µm, de préférence entre 0,4 µm et 3 µm, plus préférentiellement entre 0,5 µm et 2 µm.

12. Procédé selon l'une quelconque des revendications précédentes, dans lequel ledit liant dans ladite composition est compris entre 1 et 100 g/L, de préférence entre 10 et 80 g/L, plus préférentiellement entre 30 et 70 g/L, encore plus préférentiellement entre 35 et 60 g/L.

13. Procédé selon l'une quelconque des revendications précédentes, dans lequel ladite composition comprend en outre au moins un agent éclaircissant, de préférence du stilbène ou un dérivé du stilbène, plus préférentiellement un acide triazine stilbène disulfonique, ou un dérivé de celui-ci.

14. Procédé selon la revendication 13, dans lequel la quantité dudit agent éclaircissant dans ladite composition est comprise entre 5 et 40 g/L, de préférence entre 10 et 35 g/L, plus préférentiellement entre 15 et 30 g/L.

15. Procédé selon l'une quelconque des revendications 2 à 14, dans lequel ladite première température est comprise entre 90°C et 200°C, de préférence entre 100°C et 160°C, plus préférentiellement entre 110°C et 150°C.

16. Procédé selon l'une quelconque des revendications 2 à 15, dans lequel la seconde température est comprise entre 150°C et 200°C, de préférence entre 160°C et 180°C.

17. Tissu obtenu par un procédé selon l'une quelconque des revendications 1 à 16.

18. Tissu selon la revendication 17, dans lequel ledit tissu est un tissu tissé comprenant des fils de trame et de chaîne tissés ensemble, et dans lequel au moins une partie dudit dioxyde de titane et dudit liant est située dans les espaces définis par deux fils de chaîne adjacents et deux fils de trame adjacents qui flottent sur ou sous lesdits fils de chaîne.

19. Tissu selon la revendication 18, dans lequel ledit tissu est un tissu sergé, de préférence un tissu denim.

20. Tissu selon l'une quelconque des revendications 17 à 19, dans lequel ledit dioxyde de titane a une taille moyenne de particules comprise entre 0,25 µm et 4 µm, de préférence entre 0,4 µm et 3 µm, plus préférentiellement entre 0,5 µm et 2 µm.

21. Tissu selon l'une quelconque des revendications 17 à 20, dans lequel la quantité de dioxyde de titane est comprise entre 3 % et 10 % en poids du tissu, de préférence entre 6 % et 8 % en poids du poids total du tissu.

22. Tissu selon l'une quelconque des revendications 17 à 21, dans lequel la quantité dudit liant est comprise entre 0,5 % et 4 % en poids du tissu, de préférence entre 2 % et 3 % en poids du poids total dudit tissu.

23. Vêtement comprenant un tissu selon l'une quelconque des revendications 17 à 22.

24. Composition aqueuse pour le traitement d'un textile, de préférence un tissu, comprenant :
• du dioxyde de titane en une quantité comprise entre 5 et 500 g/L, de préférence entre 50 et 400 g/L, plus préférentiellement entre 75 et 300 g/L, encore plus préférentiellement entre 90 et 200 g/L ; et
• au moins un liant, de préférence un liant réticulable, en une quantité comprise entre 1 et 100 g/L, de préférence entre 10 et 80 g/L, de préférence entre 30 et 70 g/L, de préférence encore entre 35 et 60 g/L ;
dans lequel ledit liant a une température de transition vitreuse (Tg) comprise entre-30°C et 0°C, dans lequel la température de transition vitreuse (Tg) est mesurée selon la norme ASTM E1356, et/ou une dureté Shore A ≤ 30° Shore A, dans lequel la dureté Shore A est mesurée selon la norme ASTM D2240.

25. Composition selon la revendication 24, comprenant en outre au moins un agent éclaircissant en une quantité comprise entre 5 et 40 g/L, de préférence entre 10 et 35 g/L, plus préférentiellement entre 15 et 30 g/L.

26. Utilisation d'une composition selon la revendication 24 ou 25 dans le procédé selon l'une quelconque des revendications 1 à 16.
